

Patented Nov. 28, 1933

1,937,334

# UNITED STATES PATENT OFFICE

1,937,334

## STEEL ALLOY AND ARTICLES MADE THEREFROM

Joseph V. Emmons, Shaker Heights, Ohio, assignor to The Cleveland Twist Drill Company, Cleveland, Ohio, a corporation of Ohio

No Drawing. Application August 20, 1932  
Serial No. 629,745

25 Claims. (Cl. 75—1)

This invention relates as indicated, in general, to alloy steels in which molybdenum is employed as a principal alloying constituent. More specifically, this invention relates to that type of alloy steels which is employed in the formation of cutting tools and wear-resisting parts and is commonly referred to by those familiar with the art as an alloyed tool steel.

As is well known to those familiar with the art, 10 alloyed tool steels have, in the past, been made with tungsten as the principal alloying constituent and the types commonly known as high-speed steels are, at present, the standard commercial tool steels for high duty machining of metallic 15 substances. The tungsten high-speed steel most widely used commercially, at the present time, is essentially an alloy of carbon and iron with approximately 18% tungsten, 4% chromium and 1% vanadium. In addition, such steel contains 20 minor quantities of such alloys and impurities as manganese, silicon, copper, sulphur, phosphorus, arsenic, tin, etc. Such elements as cobalt, nickel, uranium and tantalum are sometimes added to secure certain changes in the properties of such 25 steel. This type of steel containing 18% tungsten is referred to herein as a high alloy steel. A low alloy tungsten steel in common use is an alloy of carbon and iron with approximately 4% tungsten, .75% chromium and .20% vanadium, together 30 with the usual quantities of minor alloying elements and impurities.

It has been suggested in the prior art to make high-speed steels in which molybdenum is employed as the principal alloying constituent in 35 place of tungsten. It has likewise been suggested in the prior art to replace a part of the tungsten by molybdenum. Such high-speed steels made with molybdenum and tungsten and with molybdenum without tungsten, have usually been made 40 by following the theory that molybdenum may be universally substituted for tungsten according to some definite ratio of which the following are examples:

- 45 1 molybdenum to 1.3 tungsten  
1 molybdenum to 2 tungsten  
1 molybdenum to 3 tungsten  
1 molybdenum to 4 tungsten

Upon a careful consideration of all of these 50 proposed ratios, some authorities have concluded that the proper ratio is 1 part molybdenum to 2 parts tungsten which corresponds approximately to the relation of the atomic weights of these elements. If this theory of full equivalency according to the most popular ratio of 1 part molyb-

denum to 2 parts tungsten were true, it would be possible to produce a series of high-speed steels such as are set out in the table below, which would be substantially identical as to their cutting properties. In this table all alloying elements 60 except tungsten and molybdenum are assumed to be always present in the customary quantities.

| Tungsten | Molybdenum | Tungsten equivalent | 65 |
|----------|------------|---------------------|----|
| Percent  | Percent    | Percent             |    |
| 18       | 0          | 18                  |    |
| 16       | 1          | 18                  |    |
| 14       | 2          | 18                  |    |
| 12       | 3          | 18                  |    |
| 10       | 4          | 18                  |    |
| 8        | 5          | 18                  |    |
| 6        | 6          | 18                  |    |
| 4        | 7          | 18                  |    |
| 2        | 8          | 18                  |    |
| 0        | 9          | 18                  |    |

70 The term "tungsten equivalent" as used in this description indicates the amount of actual tungsten present, if any, plus the product of the molybdenum content and a particular ratio in which molybdenum is assumed to be equivalent 80 to tungsten for the purpose under consideration.

From the literature comprising the printed prior art, it does not appear that this field has yet been completely explored, i. e., no published results have been found indicating that tests have 85 been conducted on steels having all of the variations of molybdenum and tungsten as set out in the above table. The specific compositions recorded in the prior art have generally contemplated the complete replacement of the tungsten 90 by the molybdenum. Some cases are of record where relatively small additions of molybdenum have been made to high-speed steels where tungsten is the principal alloying constituent. Such steels are, however, not pertinent to the present 95 invention for the reason that they are essentially high tungsten steels; whereas, this invention relates specifically to steels in which molybdenum is present in amounts greater than the amount of tungsten present, or steels in which molybdenum 100 is a principal alloying element

105 The type of high-speed tool steel in which tungsten has been completely replaced by molybdenum has been reported by some investigators to be lower in cutting quality, more brittle, more subject to firecracking and more erratic in performance than the standard tungsten steels. The general prevailing opinion among those familiar with the operation of high-speed steels, that the molybdenum high-speed steels are less satisfac- 110

tory than the tungsten steels, is confirmed by the fact that molybdenum high-speed steels have been employed in industry to only an insignificant degree.

5 It is also known to those familiar with the art that proposals have been made to replace tungsten by molybdenum in low alloy steels and such low alloy steels are, at present, an article of commerce. Low alloy steels have also been made in 10 which both molybdenum and tungsten have been employed in approximately equal proportions.

I have found, upon investigation and by experimental results that molybdenum tool steels free from tungsten made according to the compositions as taught in the prior art have a cutting quality materially inferior to that of comparable steels in which tungsten is the principal alloy. This has been a confirmation of the results obtained by some previous investigators of these types of steels. I have also found differences in the mechanical properties and in the microstructure of the two types of steel which indicate some of the reasons for the lack of commercial popularity of the molybdenum type.

25 A careful study of these deficiencies of the molybdenum tool steels made according to the suggestions of the prior art, and of the theories which could explain such deficiencies, has led to the discovery that steels of identical tungsten equivalents formed by combinations of various amounts of tungsten and molybdenum according to one of the previously suggested ratios do not always show identical mechanical properties or cutting quality. Different ratios have also been found to produce different results.

35 My invention, therefore, relates to the discovery that different embodiments of the ratios of molybdenum and tungsten as shown by the prior art produce different results and more specifically, to the discovery of a certain relationship between tungsten and molybdenum which, within certain limits, produces unexpectedly favorable results.

40 It is among the objects of my invention to provide a high-speed tool steel of the molybdenum type having cutting properties equal to or better than the cutting properties of the standard tungsten high-speed tool steel. Other objects of my invention will appear as the description proceeds.

50 To the accomplishment of the foregoing and related ends, said invention, then, consists of the means hereinafter fully described and particularly pointed out in the claims.

55 The following description sets forth in detail some approved combinations of ingredients embodying my invention, such disclosed means constituting, however, but a few of the various forms in which the principle of the invention may be used.

60 My invention may be, as above indicated, stated in general terms as comprising the discovery that if a specified proportional relationship, within certain limits, is maintained between the tungsten and molybdenum constituents of the alloy, a steel having unexpectedly favorable cutting and wearing properties is produced.

65 More particularly, I have found that in a steel of which molybdenum is a principal alloying constituent, the addition of auxiliary tungsten to the amount of approximately one quarter of the molybdenum present greatly and unexpectedly increases the cutting and wearing quality of tools made from such steel. This increase 70 in the cutting and wearing quality is manifested

in tool steels of both the high-speed type and the low alloy type. Further investigation has shown that there is a range of tungsten contents as calculated on the basis of the amount of molybdenum present where cutting and wearing quality in excess of that observed in tungsten-free molybdenum steels is obtained. This range of desired tungsten contents is from one twentieth to two fifths (from 5% to 40%) of the amount of the molybdenum present.

80 Steels made in the above identified range of 85 compositions also show improvements in their microscopic structure, in their mechanical properties and in the uniformity of their behavior in tools over other steels in which molybdenum is the principal alloying constituent. It has been found that tools made from steels of this type take an excellent nitrided case. They are also useful as auxiliary members of composite tools employing sintered carbide or other hard metal 95 alloys.

90 The wear-resisting properties as demonstrated in the cutting tests have been such that a wide usefulness in other fields than cutting tools may be expected, for example, in bearings and machine parts subject to wear.

100 In general, the invention contemplates an alloy involving the following components:

|            | Per cent     |
|------------|--------------|
| Carbon     | 105          |
| Manganese  | 0.5 to 1.3   |
| Silicon    | 0.1 to 1.0   |
| Chromium   | 0.1 to 0.5   |
| Tungsten   | 0.2 to 5.0   |
| Vanadium   | 0.2 to 4.0   |
| Molybdenum | 110          |
|            | 0.1 to 1.5   |
|            | 0.6 to 10.00 |

The balance being iron together with such impurities as are usual in alloy steels.

115 The foregoing table of ranges is given merely to show a characteristic range of percentages, but from the ensuing description of this invention it will be found that the actual range of percentages in which the several components may be present is, in certain instances, considerably broader than above indicated.

120 Some specific compositions of steels in which molybdenum is the principal alloying element and which contain auxiliary tungsten in the above mentioned range are as follows:

|            | Per cent |
|------------|----------|
| Carbon     | 0.61     |
| Manganese  | 0.23     |
| Silicon    | 130      |
| Chromium   | 0.29     |
| Tungsten   | 3.65     |
| Vanadium   | 1.69     |
| Molybdenum | 1.00     |
|            | 6.67     |
|            | 135      |

the balance being iron, together with such impurities as are usual in alloy steel.

140 This steel possesses properties which approach those of high-speed steel, although the amount of alloy present is much less than is usually employed in such steels. With this composition, a hardening temperature as high as 2200° F. may be employed together with drawing temperatures up to 1150° F. Tools made from this steel such as twist drills, possess great strength and cutting quality, these properties being well maintained at operating temperatures up to red heat.

145 A specific alloy steel composition which has 150

been characterized by excellent results contains the following:

|               | Percent |
|---------------|---------|
| Carbon        | 1.04    |
| 5 Manganese   | 0.17    |
| Silicon       | 0.23    |
| Chromium      | 1.15    |
| Tungsten      | 0.38    |
| Vanadium      | 0.22    |
| 10 Molybdenum | 1.55    |

the balance being iron, together with such impurities as are usual in alloy steels. Such a steel withstands hardening temperatures as high as 2000° F. without a prohibitive coarsening of the grain and retains hardness and cutting quality after drawing temperatures as high as 1100° F. It is also easy to machine, being particularly much more readily machined than known alloy steels containing high silicon. Articles made up of such alloy are readily nitrided, and because of the ability to withstand a drawing temperature above that at which a nitriding is effected, it becomes possible to apply a nitrided case to a hardened part and still retain in it a usable degree of hardness, strength and cutting quality. This unique result makes particularly possible new combinations of properties in such articles as tools, and the bodies and auxiliary wearing and cutting parts of composite tools, for instance, those utilizing a hard metal alloy, as tungsten-carbide. With such articles as twist drills, reamers, and the like, this steel provides great toughness and cutting ability, being able to continue cutting even at operating temperatures as high as 800° F.

A specific high-speed steel composition is as follows:

|            | Percent |
|------------|---------|
| 40 Carbon  | 0.78    |
| Chromium   | 5.25    |
| Tungsten   | 2.06    |
| Vanadium   | 1.01    |
| Molybdenum | 8.18    |

45 the balance being iron, together with such other alloying elements and impurities as are usually found in high-speed steel. This steel, when hardened at 2235° F. and tempered at 1040° F. has excellent hardness and strength with fair toughness. Its cutting quality has been found to be materially above that of any molybdenum high-speed steel (free from tungsten) previously examined and also to be above that of a commercial type of 18% tungsten steel with which comparisons were made.

A further satisfactory composition is as follows:

|            | Percent |
|------------|---------|
| 60 Carbon  | 0.76    |
| Chromium   | 3.82    |
| Tungsten   | 1.67    |
| Vanadium   | 1.01    |
| Molybdenum | 11.05   |

65 the balance being iron, together with such other alloying elements and impurities as are usual in high-speed steels. This steel when hardened at 2235° F. and tempered at 940° F. has hardness and strength, together with excellent toughness.

70 Its cutting quality is also materially better than that of the other molybdenum high-speed steels (free from tungsten) previously examined and was slightly better than that of the commercial type of 18% tungsten high-speed steel with which 75 it has been compared.

Tools made from steels of the above specified compositions have been found to be uniform in quality, to possess adequate toughness and to have a satisfactory freedom from firecracking.

It is believed that the limits of composition in which the useful combinations of properties may be found, may be extended beyond those used in the specific compositions above recited, if certain precautions are observed.

For example, in the high-speed steels, molybdenum contents of from 6% to 15% are contemplated but it is recognized that molybdenum even in excess of 15% may be found useful if the carbon content is also increased in the proper proportions. The chromium may be varied between limits so wide as to approach zero on the low side and ten percent. on the high side. The vanadium may also range from zero to five percent. or higher if such a balance is maintained with the carbon content that the steel will harden when quenched from a suitable temperature. Such elements as silicon, cobalt, nickel, manganese, tantalum and uranium may be included if desired to produce useful variations in the physical properties of the steel and the term "the balance being substantially iron" when used herein is intended to include, in addition to iron, minor amounts of such elements. In all such variations it is understood that a secondary amount of tungsten is to be employed for its auxiliary effect upon the principal alloying element molybdenum.

From the foregoing description, it will be apparent that my invention relates not to the substitution of molybdenum for tungsten in high-speed tool steels, as has been the practice in certain instances in the prior art, but instead to the production of a new type of molybdenum steel in which a specified minor amount of tungsten is used for its powerful auxiliary effect in increasing the cutting and wearing qualities of such steel. By the addition of the auxiliary quantities of tungsten in the specified ratio to the amount of molybdenum present, I have been able to produce a high-speed steel of the molybdenum type having cutting properties better than those of the tungsten-free molybdenum steels of the prior art and equal to or better than tungsten high-speed steels free from molybdenum with which comparisons have been made. In a similar manner I have been able to produce a low alloy molybdenum tool steel superior in cutting quality to the tungsten-free low alloy molybdenum tool steels previously known and also superior in some respects to the low alloy tungsten steels in common use.

As is well known to those familiar with the art, any specification for a particular alloying composition must permit of certain variations due to the fact that in making up the steel it is extremely difficult, if not impossible, to commercially produce a composition exactly like a given specification. It is to be understood, therefore, that throughout the description and claims where I have used figures to denote definite amounts and ranges, such amounts and ranges are to be construed to include the range of variations usually permissible in making up steel to given specifications.

This application is a continuation-in-part of 145 my co-pending application, Ser. No. 484,246, filed September 24, 1930.

Other forms may be employed embodying the features of my invention instead of the one here explained, change being made in the form or 150

construction, provided the elements stated by any of the following claims or the equivalent of such stated elements be employed.

I, therefore, particularly point out and distinctly claim as my invention:

5 1. A steel alloy of the class in which molybdenum is a principal alloying element, comprising about 0.50% to about 1.30% carbon; about 0.20% to about 10.00% chromium; about 6.00% to about 10. 15.00% molybdenum; tungsten from about 5% to about 40% of the amount of molybdenum present, and the remainder being substantially iron.

15 2. A steel alloy of the class in which molybdenum is a principal alloying element, comprising about 0.50% to about 1.30% carbon; about 0.20% to about 10.00% chromium; about 6.00% to about 15.00% molybdenum; about 0.20% to about 6.00% tungsten, the amount of such tungsten being from about 5% to about 40% of the 20 amount of molybdenum present; and the remainder being substantially iron.

25 3. A steel alloy of the class in which molybdenum is a principal alloying element, comprising about 0.50% to about 1.30% carbon; about 0.20% to about 10.00% chromium; about 0.60% to about 15.00% molybdenum; about 0.10% to about 0.45% silicon; tungsten from about 5% to about 40% of the amount of molybdenum present, such tungsten amounting to at least 0.20% of the total composition; and the remainder being substantially iron.

30 4. A steel alloy of the class in which molybdenum is a principal alloying element, comprising about 0.50% to about 1.30% carbon; about 0.20% to about 10.00% chromium; about 0.60% to about 15.00% molybdenum; about 0.10% to about 0.45% silicon, about 0.20% to about 6.00% tungsten, the amount of such tungsten being from about 5% to about 40% of the amount of 40 molybdenum present; and the remainder being substantially iron.

45 5. A steel alloy of the class in which molybdenum is a principal alloying element, comprising about 0.50% to about 1.30% carbon; about 0.20% to about 10.00% chromium; about 6.00% to about 15.00% molybdenum; tungsten from about 10% to about 30% of the amount of molybdenum present; and the remainder being substantially iron.

50 6. A steel alloy of the class in which molybdenum is a principal alloying element, comprising about 0.50% to about 1.30% carbon; about 0.10% to about 0.45% silicon; about 0.20% to about 10.00% chromium; about 0.60% to about 15.00% molybdenum; tungsten from about 10% to about 30% of the amount of molybdenum present, such tungsten amounting to at least 0.20% of the total composition; and the remainder being substantially iron.

65 7. A steel alloy of the class in which molybdenum is the alloying element having the dominating effect, comprising about 0.50% to about 1.30% carbon; about 0.20% to about 5.25% chromium; about 0.60% to about 15.00% molybdenum; tungsten from about 10% to about 30% of the amount of molybdenum present, such tungsten amounting to at least 0.38% of the total composition; and the remainder being substantially iron.

70 8. A steel alloy of the class in which molybdenum is the alloying element having the dominating effect, comprising about 0.50% to about 1.30% carbon; about 0.20% to about 5.25% chromium; about 0.60% to about 6.00% molybdenum; tungsten from about 10% to about 30%

of the amount of molybdenum present, such tungsten amounting to at least 0.38% of the total composition; and the remainder being substantially iron.

9 9. A steel alloy comprising about 0.50% to about 1.30% carbon; about 0.20% to about 5.25% chromium; about 6.00% to about 15.00% molybdenum; tungsten from about 10% to about 30% of the amount of molybdenum present; and the remainder being substantially iron.

10 10. A steel alloy comprising about 0.50% to about 1.30% carbon; about 0.20% to about 5.25% chromium; about 6.00% to about 15.00% molybdenum; tungsten about 0.60% to about 4.00%, the amount of such tungsten being from about 10% to about 30% of the amount of molybdenum present; and the remainder being substantially iron.

11 11. A steel alloy of the class in which molybdenum is a principal alloying element, comprising about 0.50% to about 1.30% carbon; about 0.20% to about 5.25% chromium; about 0.60% to about 15.00% molybdenum; tungsten from about 10% to about 30% of the amount of molybdenum present, such tungsten amounting to at least 0.38% of the total composition; about 0.10% to about 0.45% silicon, and the remainder being substantially iron.

12 12. A steel alloy of the class in which molybdenum is the alloying element having the dominating effect, comprising about 0.50% to about 1.30% carbon; about 0.20% to about 5.25% chromium; about 0.60% to about 15.00% molybdenum, tungsten from about 10% to about 30% of the amount of molybdenum present, such tungsten amounting to at least 0.38% of the total composition; about 0.10% to about 0.45% silicon; and the remainder being substantially iron.

13 13. A steel alloy of the class in which molybdenum is the alloying element having the dominating effect, comprising about 0.50% to about 1.30% carbon; about 0.20% to about 5.25% chromium; about 0.60% to about 15.00% molybdenum; tungsten from about 10% to about 30% of the amount of molybdenum present, such tungsten amounting to at least 0.38% of the total composition; at least a trace up to about 5.00% vanadium; and the remainder being substantially iron.

14 14. A steel alloy of the class in which molybdenum is the alloying element having the dominating effect, comprising about 0.50% to about 1.30% carbon; about 0.20% to about 5.25% chromium; about 0.60% to about 15.00% molybdenum; tungsten from about 10% to about 30% of the amount of molybdenum present; such tungsten amounting to at least 0.38% of the total composition; about 0.10% to about 0.45% silicon; at least a trace up to about 5.00% vanadium; and the remainder being substantially iron.

15 15. A steel alloy of the class in which molybdenum is the alloying element having the dominating effect, comprising about 0.50% to about 1.30% carbon; about 0.20% to about 5.25% chromium; about 0.60% to about 15.00% molybdenum; tungsten from about 10% to about 16% of the amount of molybdenum present, such tungsten amounting to at least 0.38% of the total composition; and the remainder being substantially iron.

16 16. A steel alloy of the class in which molybdenum is the alloying element having the dominating effect, comprising about 0.50% to about 1.30% carbon; about 0.20% to about 5.25% chromium; about 0.60% to about 6.00% molybdenum; tungsten from about 10% to about 30%

denum; tungsten about 0.38% to about 1.80%, the amount of such tungsten being from about 10% to about 30% of the amount of molybdenum present; and the remainder being substantially iron.

17. A steel alloy of the class in which molybdenum is the alloying element having the dominating effect, comprising about 0.50% to about 1.30% carbon; about 0.20% to about 5.25% chromium; about 0.60% to about 15.00% molybdenum; tungsten about 15.10% of the amount of molybdenum present and amounting to at least 0.38% of the total composition; and the remainder being substantially iron.

18. A steel alloy of the class in which molybdenum is the alloying element having the dominating effect, comprising about 0.50% to about 1.30% carbon; about 0.20% to about 5.25% chromium; about 0.60% to about 15.00% molybdenum; tungsten from about 16% to about 25% of the amount of molybdenum present and amounting to at least 0.38% of the total composition; and the remainder being substantially iron.

19. A steel alloy of the class in which molybdenum is the alloying element having the dominating effect, comprising about 0.50% to about 1.30% carbon; about 0.20% to about 5.25% chromium; about 0.60% to about 15.00% molybdenum; tungsten about 24.5% of the amount of molybdenum present and amounting to at least 0.38% of the total composition; and the remainder being substantially iron.

20. A steel alloy of the class in which molybdenum is the alloying element having the dominating effect, comprising about 0.50% to about 1.30% carbon; about 0.20% to about 5.25% chromium; about 0.60% to about 15.00% molybdenum; tungsten from about 25% to about 30%

of the amount of molybdenum present and amounting to at least 0.38% of the total composition; and the remainder being substantially iron.

21. A steel alloy of the class in which molybdenum is the alloying element having the dominating effect, comprising about 0.50% to about 1.30% carbon; about 0.20% to about 5.25% chromium; about 0.60% to about 15.00% molybdenum; tungsten about 25.34% of the amount of molybdenum present and amounting to at least 0.38% of the total composition; and the remainder being substantially iron.

22. An alloy steel containing about .76% to .8% carbon, about 3.82% to 3.91% chromium, about .25% to .5% manganese, about 7.76% to 11.05% molybdenum, about .35% to .5% silicon, about 1.01% to 1.11% vanadium, tungsten from about 15% to 23% of the amount of molybdenum present, and the balance substantially all iron.

23. A steel alloy, comprising about 0.76% carbon; about 3.82% chromium; about 11.05% molybdenum; about 1.67% tungsten; about 1.01% vanadium; and the remainder being substantially iron.

24. An article of manufacture embodying an alloy consisting of carbon about 1.04%, manganese about 0.17%, silicon about 0.23%, chromium about 1.15%, tungsten about 0.38%, vanadium about 0.22%, molybdenum about 1.55%, the remainder being substantially iron.

25. An article of manufacture embodying an alloy consisting of carbon about 0.61%, manganese about 0.22%, silicon about 0.29%, chromium about 3.65%, tungsten about 1.69%, vanadium about 1.00%, molybdenum about 6.67%, the remainder being substantially iron.

JOSEPH V. EMMONS.

40

115

45

120

50

125

55

130

60

135

65

140

70

145

75

150